

March 11, 1941.

H. E. FEIST

2,234,237

COATING

Filed Oct. 31, 1936



Fig. 1.

Fig. 2.



Fig. 3.



Fig. 4.



INVENTOR:  
HERBERT E. FEIST.

by *H. E. Feist*  
ATTORNEY

## UNITED STATES PATENT OFFICE

2,234,237

## COATING

Herbert E. Feist, New York, N. Y.

Application October 31, 1936, Serial No. 108,611

1 Claim. (Cl. 91—68)

My invention relates to the finishing of the surface of objects of any kind, and more particularly to a coating material adapted to be applied to backings of any kind, such as to surfaces of walls, wallboards, woodwork, potteries, metals and other materials and to a method for the production of decorating coatings on said surfaces.

One of the objects of my invention is to provide 10 a non-inflammable coating material, which in plastic condition is applied to a surface, may be provided with a relief design while being in plastic condition and dries and hardens in the air in such a way, that prior to the drying the mass applied 15 to the surface smooths to a certain degree, so that the final relief has no sharp ridges or peaks.

Another object of my invention is to provide 20 a plastic coating material, which after the hardening results in a solid mass having minute pores throughout and may be burnished under the 25 application of pressure.

Still another object of my invention is to provide methods to apply and permanently secure a metallic covering to parts or the entire surface 25 of a coating applied to a backing, such as the surface of a wall, wallboard, woodwork, metals, 30 potteries and other materials in a manner, which may be carried out by any person without difficulties.

30 A further object of my invention consists in the production of metallized or gilded picture frames, whereby the hitherto necessary plurality of intermediate layers, which substantially consist of a mixture of gypsum and glue, and the layer of a polishable material or materials may be omitted, so that the expenses for the production are considerably decreased and minimized.

In order to carry out my invention into practice, I mix ground minerals consisting of one 40 or a plurality of the following groups as silicates, volcanic minerals or calcareous minerals, with binding means containing at least two different glues. Preferably, the minerals used have different sizes of grain and degree of hardness. The 45 addition of water to such a mixture results in a plastic mass, which may be applied to the backing either by hand or by a mechanical process. By means of suitable tools, such as a brush, a comb, a roller, a sponge, a spatula or the like, a relief 50 design may be imparted to the plastic coating being still wet, if desired. On exposure to air the coating dries and hardens thereby enhancing the strength of the material or the object, to 55 which it is applied. The hardened mass has minute and hardly visible pores or interstices

throughout and is pliable to a certain degree, so that it may be applied to backings of metal, wood-work, fibre-board and may withstand small changes of the length of the surface of such backings. Furthermore, the mass is fire-resistant. The hardened coating may be burnished under application of pressure, whereby the above mentioned minute pores on the surface will be closed and the surface obtains a high-glossy appearance. While the thus treated mass may form 10 the final coating of an object or article, still more attractive and new effects may be obtained, if the hardened mass is used as an intermediate layer and a covering of metal particles is deposited thereon and secured thereto. Said covering or 15 finishing may be applied either to the entire surface of the intermediate layer or to parts thereof only, for example to the projecting or raised parts of the relief. Hereinafter I describe several methods for the production of coatings with coverings, 20 whereby the term "metallized coating" shall indicate, that the coating is provided with a metal covering.

In the accompanying drawing several embodiments of my coating are illustrated.

Fig. 1 shows a fractional top plan view of a backing, a wall for example, to the surface of which my new coating provided with a relief design is applied.

Fig. 2 shows a cross-sectional view of the backing, taken on line 2—2 of Fig. 1.

Fig. 3 shows a cross-sectional view of a portion of the backing in an enlarged scale, illustrating the interstices or pores on the surface of the coating.

Fig. 4 shows a cross-sectional view similar to Fig. 3, whereby, however, the coating forms an intermediate layer and the surface thereof is provided with a metal covering or finishing, so that a "metallized coating" is obtained.

According to one embodiment of my invention to produce a "metallized coating," I apply the above mentioned pasty mass to the surface of a backing, such as of a wall or an article, by means of a brush or a spraying gun. Then a relief design is imparted to the plastic coating in the above mentioned manner, and the coating obtains the appearance as shown in Figs. 1 and 2. After the drying and hardening of the coating or intermediate layer a metal brush with thin 50 bristles (metal wires) of a diameter of less than .1 mm. is rubbed on the surface of the intermediate layer. The material of the bristles used for this purpose may be a metal or a metal alloy, such as gold, silver, copper, brass, bronze, nickel-silver 55

or even steel. Although the hardness of the metal or metal alloy may be higher than the average hardness of the composition forming the intermediate layer, particles of the metal are detached or rubbed off from the metal bristles during the rubbing operation by means of those mineral grains interspersed in said composition, which have a hardness higher than the hardness of the metal. The detached metal particles settle in the pores or interstices (see Fig. 3) on the surface of the mass and fill out the pores, as shown in Fig. 4. Thereupon the metal layer deposited on the intermediate layer may be polished by means of a polishing tool or burnisher under the application of pressure. The tool may be made of agate for example. During this polishing operation the detached metal particles are firmly pressed into the pores and interstices of the surface of the mass and displaced in such a way, that they form a covering or finishing, which has the appearance of an uninterrupted, smooth and bright metal covering.

Another method to metallize a part or the whole of the surface of the hardened intermediate layer consists therein, that a round piece of metal is rubbed on the surface of the layer. The metal particles detached from the rod consisting of a metal or metal alloy are deposited in the pores or interstices of the surface. If the metal rod is drawn over or rubbed on the layer under the application of sufficient pressure, a special subsequent polishing operation by means of a polishing tool may be omitted, as the metal covering produced by the rod obtains a sufficient smoothness and brightness.

The coating mass and the metal covering, which are produced according to either one of the above mentioned methods, may be protected against the influence of the atmosphere by a protecting or decorating layer of varnish or lacquer thereon.

Still another method for the production of a metallized coating consists therein, that the surface of the intermediate layer applied to the backing is moistened by means of water or a liquid binder, whereupon a metal powder is rubbed on the entire moistened surface or a part thereof by means of a cloth or brush. The metal covering thus formed is polished by means of a burnisher or the like under the application of pressure. Subsequent to the polishing operation a lacquer is applied to the metal covering to protect and fix same. Instead of first moistening the surface of the intermediate layer, it is also possible to prepare a suspension of a metal powder in a suitable binder and to apply same immediately on the surface of the hardened intermediate layer without moistening same. Then the metal covering thus obtained is polished in the manner mentioned above. Finally, a protecting layer of lacquer may be applied to the metal covering, if desired. Similar to the methods mentioned in the foregoing paragraphs, these two methods may be used for the production of metallized coatings on walls, wall-boards or other material as well as on the surfaces of articles of any kind. Special advantages, however, are obtained, if these methods are applied to the production of picture frames, which have a metallic surface. According to the hitherto usual practice in the picture frame industry a considerable number of intermediate layers of a mixture of gypsum and glue are applied successively to the wooden base of the frame, whereby the uppermost layer of gypsum and glue is shaped to the desired de-

sign. Thereupon a layer of a polishable material is applied to said uppermost layer, so that the metal layer applied thereon subsequently may adhere to the intermediate layers and may be polished. According to my new methods a single intermediate layer of my composition is sufficient, and the metal covering may be applied directly thereon. Apart from the fact, that at least quite a number of steps, i. e. the application of the plurality of intermediate layers and of the layer of polishable material, are omitted and a saving on working time is obtained, my picture frame is superior to the hitherto known frames, as it consists of a hard and solid mass, while the gypsum frames are formed by a fragile and brittle mass.

A further method to produce new and attractive metallic effects on a hardened intermediate relief layer with projecting and depressed parts consists therein, that a layer of varnish, which may be colored or non-colored, is applied to the hardened intermediate layer, whereupon a metal powder is deposited on said layer of varnish by spraying, blowing or powdering thereon, while the varnish is still wet. As the powder is lighter than the varnish, the powder remains substantially on the projecting parts of the relief design, while the depressed parts are covered with varnish only, i. e. the depressed parts remain free from metal powder. While preferably the intermediate relief layer is formed by my new coating material, as it enhances the adherence of the particles of the covering to the relief layer, any other composition, which hardens, may be used.

Coloring earths, pigment colors or lake colors, which are alkali resistant to a certain degree, may be added to the mixture, if desired. Suitable coloring earths are ochre, umber and sienna for example, suitable pigment colors are cobalt-blue, ultramarine-blue, etc., and suitable lake colors are lithol-red, Hansa-yellow, etc.

An important feature of my invention is the use of minerals, which have different sizes of grain and degree of hardness. Such ground minerals may be silicates, granite, basalt or lava having a hardness of 6-8 according to the scale of hardness (Moh's scale) and a size of grain allowing 45 to 50% to pass through a sieve of 325 mesh per sq. inch, 65 to 70% to pass through a sieve of 200 mesh per sq. inch, 75 to 80% to pass through a sieve of 100 mesh per sq. inch, 95 to 100% to pass through a sieve of 50 mesh per sq. inch. Other ground minerals are limestone or chalk having a hardness of 3-5 according to the scale of hardness (Moh's scale) and a size of grain allowing 55 to 60% to pass through a sieve of 325 mesh per sq. inch, 70 to 75% to pass through a sieve of 200 mesh per sq. inch, 80 to 85% to pass through a sieve of 100 mesh per sq. inch, 100% to pass through a sieve of 50 mesh per sq. inch.

Casein, albumin, a resin emulsion or the like, and water are adapted to be used as binding means.

My invention will be illustrated by the following:

| Example          | Parts by weight |
|------------------|-----------------|
| Ground basalt    | 32              |
| Ground limestone | 27              |
| Ground lava      | 18              |
| Coloring means   | 4               |

are thoroughly mixed with each other, whereby the minerals have the size of grain and degree of hardness as mentioned above. In order to 75

bind the powdery materials, a solution is prepared, which consists of 20 parts of weight of casein mixed with 50 parts of weight of water, to which 4 parts of weight of borax dissolved in 5 10 parts of water are added. Furthermore, 2 parts of weight of resin soap produced by boiling a mixture of 10 parts of weight of resin and 2 parts of weight of calcined soda and 100 parts of weight of water are added. Such an amount 10 of the combined liquids is added to the mixture of minerals and coloring means, that a thick paste is obtained. This paste may be diluted with water, so that a mass is produced, which has a consistence permitting it to be applied on 15 a backing by means of a brush, spatula or sprayer. After the application of the mass to the backing by means of a brush, spatula or sprayer, a relief design is given to the mass, which is still in pasty condition, by means of a roller, comb, spatula, brush or any other suitable tool. 20 Then the mass is caused to harden to form a coating. After the hardening of the mass, the layer thus obtained may be metallized by either one of the above described methods.

25 I have described preferred embodiments of my invention but it is clear that numerous changes and omissions may be made without departing from the spirit of my invention.

What I claim is:

An article of manufacture having on its surface a coating comprising an intermediate layer of a hardened composition of a mixture of ground minerals, coloring matter and binding means, 5 said minerals being selected from the group consisting of silicates, volcanic minerals and calcareous minerals, the minerals used having different size of grain and degree of hardness, said binding means containing a mixture of two different glues, one of said glues being deposited from a mixture consisting of substantially 20 parts of weight of casein mixed with substantially 4 parts of weight of borax dissolved in substantially 10 parts of weight of water, the other 15 glue being deposited from a mixture consisting of substantially 2 parts of weight of a resin soap produced by boiling a mixture of substantially 10 parts of weight of resin and substantially 2 parts of weight of calcined soda and substantially 20 100 parts of weight of water, and said composition having interstices on the surface, and a top layer of metal particles, said top layer being anchored in said interstices of said intermediate 25 layer.

HERBERT E. FEIST.